

## UNITED STATES PATENT OFFICE

2,567,456

METAL CLEANING COMPOSITION AND  
PROCESSHugh Graham Webster, Detroit, Mich., assignor.  
to J. H. Shoemaker, Detroit, Mich.No Drawing. Application April 7, 1947,  
Serial No. 739,961

4 Claims. (Cl. 134—3)

1

This application relates to metal cleaning and particularly to a process and a composition of matter for cleaning metallic objects having large quantities of organic materials to be removed. Examples might be the cleaning of cast iron motor blocks of automobiles which have long been in use. Such blocks are usually encrusted with large quantities of road dirt, grease, oil, etc.

The first step of the process is an immersion of the article to be cleaned in a non-electrolytic bath comprising a molten mixture of approximately nineteen parts by weight of an alkali metal nitrate, such as sodium nitrate, nineteen parts by weight of an alkali metal hydroxide, such as sodium hydroxide, and one part by weight of an alkali metal chloride, such as sodium chloride, the latter being preferably in flake form. The immersion may be of any desired length, just so long as it is sufficient to remove the organic surface impurities, such as those above described and to convert inorganic surface impurities, such as sulphur, carbon, etc. to oxide form. The operating temperature of the bath may be any desired temperature, just so long as it is above the melting point of the molten mixture. In the proportions specified above, the melting point is approximately 550° F.

The second step of the process comprises immersing the metal removed from the first bath in a second non-electrolytic bath which is of such a nature that when the metal article is immersed in the second bath for any desired and proper time, a chemical reaction will take place between the composition of the bath and the oxidized coating which will remove such oxidized coating from the metal object and thus leave the surface free of the original impurities, the organic impurities of which had been removed, and the inorganic impurities of which had been transformed into oxides now being removed by the second bath.

The immersion in the second bath, however, is of such short duration as not to etch the surface and thus to expose at the surface other impurities, not previously existent, or not previously exposed. The second bath leaves the surface free of all impurities and consisting solely of the metal. The second bath is preferably a dilute acid selected from the class of hydrochloric and sulphuric acids and the immersion in such second bath is extremely brief.

It may be mentioned that each step hereof is followed by a water rinse, but since water rinsing

2

is so ordinary and well known a practice, it is not here considered as a step in the process.

It may be mentioned that an important difference between the bath hereof and the bath of a prior application, Serial No. 520,332, now Patent 2,458,661, patented January 11, 1949, is that the bath hereof contains a considerably larger proportion of sodium nitrate. I believe that such excess of sodium nitrate is used up in converting the organic material, above described, to carbon dioxide, which enters the bath as a carbonate and may thus be removed. It has been found that when using a bath of the prior application, Serial No. 520,332, on automobile engine blocks which have been in use a long time, and are coated with dirt, grease, oil, etc., that after several weeks of use of such bath with such objects, the composition of the bath had deteriorated to the point where it was no longer effective. The excess of nitrate represented by the formula herein disclosed, overcomes the weakening of the bath of the prior application when used for the special type of objects being cleaned as here described — namely, objects coated with large amounts of organic materials, such as oil, grease, road dirt, etc.

Now having described the process herein disclosed, reference should be had to the claims which follow.

I claim:

1. Descaling and degreasing composition for grease and scale coated alkali resistant metals for use in molten bath form comprising a mixture of about nineteen parts by weight of alkali metal hydroxide, about nineteen parts by weight of alkali metal nitrate and about one part by weight of alkali metal chloride.
2. Descaling and degreasing composition for grease and scale coated alkali resistant metals for use in molten bath form comprising a mixture of about nineteen parts by weight of sodium hydroxide, about nineteen parts by weight of sodium nitrate and about one part by weight of sodium chloride.
3. A two step non-electrolytic process for cleaning the surfaces of alkali resistant metals, having substantial amounts of oxidizable organic materials thereon, such as oils, greases etc., as well as oxidized portions of the metal, such as scale etc., to be removed, wherein each step is in the nature of a chemical reaction, and wherein the second step leaves no added finish to the surface, and wherein the first step comprises immersing the metal in a bath comprising a molten mixture of approximately 19 parts by weight of

alkali metal nitrate, approximately 19 parts by weight of alkali metal hydroxide and approximately 1 part by weight of alkali metal chloride, for a period of time sufficient to remove any organic surface impurities and convert inorganic surface impurities to an oxidized coating, more readily soluble than were the original inorganic impurities, the operating temperature of the first bath being above the melting point of the molten mixture, and wherein the second step comprises immersing the metal in a bath of a dilute acid selected from the class consisting of hydrochloric and sulphuric acids, whereby when the metal is immersed therein for a proper period of time, the bath will react chemically with the oxidized coating to remove it, so as to leave the surface free of the original impurities and of the oxidized coating as well, the second step, however, being such as not to expose at the surface other impurities, not previously existent, or not previously exposed, thus leaving the surface free of all impurities and consisting solely of the metal, the immersion in the second bath being sufficiently brief so as not to permit the acid to attack the metal, but merely to remove the oxidized coating formed by the first step.

4. A two step non-electrolytic process for cleaning the surfaces of alkali resistant metals, having substantial amounts of oxidizable organic materials thereon, such as oils, greases, etc., as well as oxidized portions of the metal, such as scale, etc., to be removed, wherein each step is in the nature of a chemical reaction, and wherein the second step leaves no added finish to the surface, and wherein the first step comprises immersing the metal in a bath comprising a molten mixture of approximately 19 parts by weight of sodium nitrate, approximately 19 parts by weight of sodium hydroxide and approximately 1 part by weight of sodium chloride, for a period

5 of time sufficient to remove any organic surface impurities and convert inorganic surface impurities to an oxidized coating, more readily soluble than were the original inorganic impurities, the operating temperature of the first bath being above the melting point of the molten mixture, and wherein the second step comprises immersing the metal in a bath of a dilute acid selected from the class consisting of hydrochloric and sulphuric acids, whereby when the metal is immersed therein for a proper period of time, the bath will react chemically with the oxidized coating to remove it, so as to leave the surface free of the original impurities and of the oxidized coating as well, the second step, however, being such as not to expose at the surface other impurities, not previously existent, or not previously exposed, thus leaving the surface free of all impurities and consisting solely of the metal, the immersion in the second bath being sufficiently brief so as not to permit the acid to attack the metal, but merely to remove the oxidized coating formed by the first step.

25

30

35

40

HUGH GRAHAM WEBSTER.

## REFERENCES CITED

The following references are of record in the file of this patent:

## UNITED STATES PATENTS

| Number    | Name           | Date          |
|-----------|----------------|---------------|
| 2,244,526 | Mackay         | June 3, 1941  |
| 2,311,099 | Tainton        | Feb. 16, 1943 |
| 2,380,284 | Young          | July 10, 1945 |
| 2,395,694 | Spence         | Feb. 26, 1946 |
| 2,458,661 | Webster et al. | Jan. 11, 1949 |

## FOREIGN PATENTS

| Number  | Country       | Date         |
|---------|---------------|--------------|
| 466,661 | Great Britain | May 26, 1937 |